# EUROPEAN PATENT SPECIFICATION

(11) **EP 2 321 451 B1**
(45) Date of publication and mention of the grant of the patent: **19.12.2018**
(21) Application number: 09792294.2
(22) Date of filing: 08.09.2009
(51) Int. Cl.: D01D 5/00

(54) **HIGH THROUGHPUT ELECTROBLOWING PROCESS**
HOCHLEISTUNGSELEKTROBLASVERFAHREN
PROCESSUS D'ÉLECTROSOUFFLAGE À FORT RENDEMENT

(30) Priority: 05.09.2008 US 191102 P
(43) Date of publication of application: 18.05.2011
(73) Proprietor: E. I. du Pont de Nemours and Company, Wilmington, DE 19898 (US)
(72) Inventor: DEE, Gregory, T., Wilmington Delaware 19802-2652 (US); HOVANEC, Joseph, Brian, Richmond Virginia 23223 (US); MEERVELD, Jan, Van, NL-L-1137 Howald (NL)
(74) Representative: Dannenberger, Oliver Andre
(86) International application number: PCT/US2009/056157
(87) International publication number: WO 2010/028326

(56) References cited:
- WO-A1-2006/066025
- WO-A1-2007/022390
- US-A1- 2005 073 075
- US-A1- 2006 097 431
- US-B1- 6 520 425
- ZHENG-MING HUANG ET AL: "A review on polymer nanofibers by electrospinning and their applications in nanocomposites" COMPOSITES SCIENCE AND TECHNOLOGY, ELSEVIER, UK, vol. 63, no. 15, 2 July 2003 (2003-07-02), pages 2223-2253, XP002516036 ISSN: 0266-3538 [retrieved on 2003-07-02]
- UM I C ET AL: "Electro-Spinning and Electro-Blowing of Hyaluronic acid" BIOMACROMOLECULES, ACS, WASHINGTON, DC, US, vol. 5, no. 4, 5 July 2004 (2004-07-05), pages 1428-1436, XP002483474 ISSN: 1525-7797 [retrieved on 2004-07-05]

## Description

### FIELD OF THE INVENTION

The present invention relates to a process for forming a fibrous web from a high throughput electroblowing process.

### BACKGROUND

Solution spinning processes are frequently used to manufacture fibers and nonwoven fabrics, and in some cases have the advantage of high throughputs, such that the fibers or fabrics can be made in large, commercially viable quantities. These processes can be used to make fibrous webs that are useful in medical garments, filters and other end uses that require a selective barrier. The performance of these types of fibrous webs can be enhanced with the utilization of fibers with small diameters.

A type of solution spinning called electroblowing produces very fine fibers by spinning a polymer solution through a spinning nozzle in combination with a blowing gas and in the presence of an electric field.

However, it would be desirable to increase the throughput of this process to increase process efficiencies and lower the cost of manufacturing, without sacrificing fiber uniformity and product quality.

WO 2007/022390 A1 describes a fiber spinning process using an electrically conductive polymer-containing liquid stream wherein the liquid stream is either a polymer solution or a molten polymer.

### SUMMARY OF THE INVENTION

The present invention is a fiber spinning process comprising the steps of providing a polymer solution, which comprises at least one polymer dissolved in at least one solvent with a vapor pressure of at least about 6 kPa at 25°C, to a spinneret, issuing the polymer solution in combination with a blowing gas in a direction away from at least one spinning nozzle in the spinneret and in the presence of an electric field wherein the polymer solution is discharged through the spinning nozzle at a discharge rate between about 6 to about 100 ml/min/hole, forming fibers, and collecting the fibers on a collector, wherein the solvent is selected from the group consisting of pentane, hexane, heptane, cyclohexane, methylcyclohexane, and benzene.

### BRIEF DESCRIPTION OF THE DRAWINGS

The accompanying drawing, which is incorporated in and constitutes a part of this specification, and together with the description, serves to explain the principles of the invention.

Fig. 1 is a schematic of a prior art electroblowing apparatus useful for preparing a fibrous web according to the invention.

### DETAILED DESCRIPTION OF THE INVENTION

The present invention relates to solvent-spun webs and fabrics for a variety of customer end-use applications, such as filtration media, energy storage separators, protective apparel and the like.

The present invention uses an electroblowing process to spin a polymer dissolved in a high vapor pressure solvent at a high rate of throughput into fibers and webs.

The process for making a fiber layer(s) is disclosed in International Publication Number WO2003/080905 (U.S. Serial No. 10/822,325). Fig. 1 is a schematic diagram of an electroblowing apparatus useful for carrying out the process of the present invention using electroblowing (or "electro-blown spinning") as described in International Publication Number WO2003/080905. This prior art electroblowing method comprises feeding a solution of a polymer in a solvent from a storage tank 100, through a spinneret 102, to a spinning nozzle 104 to which a high voltage is applied, while compressed gas or blowing gas is directed toward the polymer solution through a blowing gas nozzle 106 as the polymer solution exits the spinning nozzle 104 to form fibers, and collecting the fibers into a web on a grounded collector 110 under vacuum created by vacuum chamber 114 and blower 112.

The collection apparatus is preferably a moving collection belt positioned within the electrostatic field between the spinneret 102 and the collector 110. After being collected, the fiber layer is directed to and wound onto a wind-up roll on the downstream side of the collector 110. Optionally, the fibrous web can be deposited onto any of a variety of porous scrim materials arranged on the moving collection belt, such as spunbonded nonwovens, meltblown nonwovens, needle punched nonwovens, woven fabrics, knit fabrics, apertured films, paper and combinations thereof.

Optionally, a secondary gas can contact the fibers downstream from the spinneret to help drive off solvent from the fiber. When electroblowing fibers with a high throughput rate, large quantities of solvent must be removed from the fiber forming polymer solution. The secondary gas can be positioned to impinge the fibers or can be used as a sweeping gas to help remove solvent from the general spinning area.

In order to spin fibers at high throughput or discharge rate, solvents with high vapor pressure can be used. According to the invention, solvents with vapor pressures of at least 6 kPa at 25°C are used, preferably of at least 10 kPa at 25°C and more preferably of at least 20 kPa at 25°C. Suitable solvents with high vapor pressure are the hydrocarbons pentane (68.3), hexane (20.2), heptane (6.1), cyclohexane (13), methylcyclohexane (6.1), and benzene (12.3), where the numbers in parentheses are the vapor pressures of these solvents at 25°C in units of kPa. The vapor pressure data was obtained from "Organic Solvents". Volume 2, fourth edition, by John Riddick, William Bunger, and Theodore Sakano, John Wiley & Sons, 1986 or from the DIPPR® database of physical properties of solvents.

The polymer solution can be spun at a temperature of about 0°C to the boiling point of the solvent.

These solvents can be used to prepare polymer solutions that can be spun at a discharge rate between 6 to 100 ml/min/hole, more advantageously between 10 to 100 ml/min/hole, and most advantageously between 20 to 100 ml/min/hole.

The polymer(s) that can be used in making fiber layers in accordance with the process of the present invention are not particularly limited, provided that they are substantially soluble in the selected solvent at the desired concentration and can be spun into fibers by the process described herein. Examples of these polymers generally include hydrocarbon polymers. Examples of hydrocarbon polymers suitable for the present invention include polyolefins, polydienes, polystyrene and blends thereof. Examples polyolefins include polyethylene, polypropylene, poly(1-butene), poly(4-methyl-1-pentene), and blends, mixtures and copolymers thereof.

In addition to the forgoing polymers, other examples include polysulfones, polycarbonates, poly(meth)acrylates, cellulose esters, polyvinylchlorides, and blends thereof. Examples of poly(meth)acrylates include polymethylacrylate and polymethylmethacrylate. Examples of cellulose esters include cellulose triacetate. Examples of polyesters include polyethylene therephthalate, polypropylene therephthalate, polybutylene therephthalate, poly(epsilon-caprolactone), poly(DL-lactic acid) and poly(L-lactide).

The blowing gas can be selected from the group of air, nitrogen, argon, helium, carbon dioxide, hydrocarbons, halocarbons, halohydrocarbons and mixtures thereof. The blowing gas is injected at a flow velocity of 50 to 340 m/sec and a temperature from about ambient to 300°C.

The fibers produced have a number average fiber diameter preferably less than 1,000 nanometers, more preferably less than 800 nanometers and most preferably less than 500 nanometers. The fibers can be continuous or discontinuous. The fibers can have an essentially round cross section shape.

The electric field can have a voltage potential of about 10 to about 100 kV. The electric field can be used to create a corona charge.

The fibers can be collected into a fibrous web comprising round cross section, weakly interacting polymer fibers having a number average fiber diameter less than about 1,000 nanometers.

The secondary gas can be selected from the group of air, nitrogen, argon, helium, carbon dioxide, hydrocarbons, halocarbons, halohydrocarbons and mixtures thereof. The secondary gas is injected at a flow velocity of 50 to 340 m/sec and a temperature from about ambient to 300°C.

### TEST METHODS

Fiber Diameter was determined as follows. Two to three scanning electron microscope (SEM) images were taken of each fine fiber layer sample. The diameter of clearly distinguishable fine fibers were measured from the photographs and recorded. Defects were not included (i.e., lumps of fine fibers, polymer drops, intersections of fine fibers). The number average fiber diameter from about 50 to 300 counts for each sample was calculated.

### EXAMPLES

The fiber examples below were prepared using the general process and apparatus described above with the specific changes as noted below.

### Example 1 (Reference Example)

A 9 wt% solution of polymethylmethacrylate (PMMA) was dissolved in acetone (vapor pressure of 24.2 kPa at 25°C) at room temperature. A magnetic stirrer was used to agitate the solution. The homogeneous solution was transferred to a sealed glass container and transported to the spin chamber. The solution was transferred into the reservoir of the spin chamber and sealed. A spinneret with a 0.254 mm inside diameter single spinning nozzle was used. A drum collector was used to collect the sample. The spinneret was placed at a negative potential of 100 kV. The collector was grounded. The distance from the spinning nozzle exit to the collector surface was 51 cm. Air was used for the blowing gas. Nitrogen was used for the secondary gas to control the relative humidity and the temperature in the spin chamber. The flow of nitrogen was sufficient to avoid the concentration of the solvent vapor in the spin chamber exceeding the lower explosion limit. The relative humidity was controlled to be less than 11%. The spin chamber temperature was close to 23 °C for the duration of the experiment. A nitrogen pressure of 0.2044 MPa was used to maintain a solution flow rate of 6.7 ml/min/hole. The blowing gas was controlled to maintain an exit velocity on the order of 67 m/sec. The blowing gas temperature was close to 23 °C. Fiber was visible in the plume soon after the solution flow was initiated. Fiber was deposited in a swath on the drum. The number average fiber diameter of the fibers was measured to be 393 nanometers.

### Example 2 (Reference Example)

A 9 wt% solution of polystyrene was dissolved in dichloromethane (vapor pressure of 58.1 kPa at 25°C) at room temperature. A magnetic stirrer was used to agitate the solution. The homogeneous solution was transferred to a sealed glass container and transported to the spin chamber. The solution was transferred into the reservoir of the spin chamber and sealed. A spinneret with a 0.406 mm inside diameter single spinning nozzle was used. A drum collector was used to collect the sample. The spinneret was placed at a negative potential of 100 kV. The collector was grounded. The distance from the spinning nozzle exit to the collector surface was 95 cm. Air was used for the blowing gas. Air was used for the secondary gas to control the relative humidity and the temperature in the spin chamber. The flow of air was sufficient to avoid the concentration of the solvent vapor in the spin chamber exceeding the lower explosion limit. The relative humidity was controlled to be less than 11%. The spin chamber temperature was close to 32 °C for the duration of the experiment. A nitrogen pressure of 0.515 MPa was used to maintain a solution flow rate of 34.3 ml/min/hole. The blowing gas was controlled to maintain an exit velocity on the order of 150 m/sec. The blowing gas temperature was close to 24 °C. Fiber was visible in the plume soon after the solution flow was initiated. Fiber was deposited in a swath on the drum. The number average fiber diameter of the fibers was measured to be 335 nanometers.

### Example 3 (Reference Example)

A 9 wt% solution of polystyrene was dissolved in dichloromethane (vapor pressure of 58.1 kPa at 25°C) at room temperature. A magnetic stirrer was used to agitate the solution. The homogeneous solution was transferred to a sealed glass container and transported to the spin chamber. The solution was transferred into the reservoir of the spin chamber and sealed. A spinneret with a 0.406 mm inside diameter single spinning nozzle was used. A drum collector was used to collect the sample. The spinneret was placed at a negative potential of 100 kV. The collector was grounded. The distance from the spinning nozzle exit to the collector surface was 114 cm. Air was used for the blowing gas. Air was used for the secondary gas to control the relative humidity and the temperature in the spin chamber. The flow of air was sufficient to avoid the concentration of the solvent vapor in the spin chamber exceeding the lower explosion limit. The relative humidity was controlled to be less than 11 %. The spin chamber temperature was close to 37 °C for the duration of the experiment. A nitrogen pressure of 0.77 MPa was used to maintain a solution flow rate of 57.1 ml/min/hole. The blowing gas was controlled to maintain an exit velocity on the order of 150 m/sec. The blowing gas temperature was close to 24 °C. Fiber was visible in the plume soon after the solution flow was initiated. Fiber was deposited in a swath on the drum. The number average fiber diameter of the fibers was measured to be 630 nanometers.

### Example 4

An 11 wt% solution of Engage 8400 (an ethylene octene copolymer), available from DuPont, was dissolved in methylcyclohexane (vapor pressure of 6.1 kPa at 25°C) using a reflux condenser. A magnetic stirrer was used to agitate the hot solution. The homogeneous solution was transferred to a sealed glass container and transported to the spin chamber. The solution was transferred into the reservoir of the spin chamber and sealed. A spinneret with a 0.4064 mm inside diameter single spinning nozzle was used. A drum collector was used to collect the sample. The spinneret was placed at a negative potential of 100 kV. The collector was grounded. The distance from the spinning nozzle exit to the collector surface was 30 cm. Air was used for the blowing gas. Nitrogen was used for the secondary gas to control the relative humidity and the temperature in the spin chamber. The flow of nitrogen was sufficient to avoid the concentration of the solvent vapor in the spin chamber exceeding the lower explosion limit. The relative humidity was controlled to be less than 9%. The spin chamber temperature was close to 29 °C for the duration of the experiment. A nitrogen pressure of 0.308 MPa was used to maintain a solution flow rate of 12.6 ml/min/hole. The blowing gas was controlled to maintain an exit velocity on the order of 156 m/sec. The blowing gas temperature was close to 28 °C. Once the solution flow was initiated, fiber was visible in the plume. Fiber was deposited in a swath on the drum. The number average fiber diameter of the fibers was measured to be 502 nanometers.

## Claims

1. A fiber spinning process comprising:
providing a polymer solution, which comprises at least one polymer dissolved in at least one solvent with a vapor pressure of at least 6 kPa at 25°C, to a spinneret;
issuing the polymer solution in combination with a blowing gas in a direction away from at least one spinning nozzle in the spinneret and in the presence of an electric field wherein the polymer solution is discharged through the spinning nozzle at a discharge rate between 6 to 100 ml/min/hole;
forming fibers; and
collecting the fibers on a collector,
wherein the solvent is selected from the group consisting of pentane, hexane, heptane, cyclohexane, methylcyclohexane, and benzene.

2. The process according to claim 1, wherein the vapor pressure is of at least 10 kPa at 25°C, or preferably of at least 20 kPa at 25°C.

3. The process according to claim 1, wherein the polymer solution is discharged through the spinning nozzle at a discharge rate between 10 to 100 ml/min/hole, or preferably between 20 to 100 ml/min/hole.

4. The process according to claim 1, wherein the blowing gas is selected from the group of air, nitrogen, argon, helium, carbon dioxide, hydrocarbons, halocarbons, halohydrocarbons and mixtures thereof.

5. The process according to claim 1, wherein the blowing gas is injected at a flow velocity of 50 to 340 m/sec and a temperature from ambient to 300°C.

6. The process according to claim 1, wherein the fibers have a number average fiber diameter less than 1000 nanometers, preferably less than 800 nanometers, more preferably less than 500 nanometers.

7. The process according to claim 1, wherein the electric field has a voltage potential of 10 kV to 100 kV.

8. The process according to claim 1, wherein the electrical field is a corona charging field.

9. The process according to claim 1, wherein the fibers have a cross section shape that is essentially round.

10. The process according to claim 1, further comprising contacting the fibers with a secondary gas located downstream from the spinneret.

11. The process according to claim 10, wherein the blowing gas is selected from the group of air, nitrogen, argon, helium, carbon dioxide, hydrocarbons, halocarbons, halohydrocarbons and mixtures thereof.

12. The process according to claim 10, wherein the blowing gas is injected at a flow velocity of about 50 to about 340 m/sec and a temperature from about ambient to about 300°C.

13. The process according to claim 1, wherein said at least one polymer in said polymer solution is selected from the group consisting of polyolefins, polydienes, polystyrene, polysulfones, polycarbonates, poly(meth)acrylates, cellulose esters, polyvinylchlorides and blends thereof.

## Patentansprüche

1. Faserspinnverfahren, umfassend:
bereitstellen einer Polymerlösung, die mindestens ein Polymer umfasst, das in mindestens einem Lösemittel mit einem Dampfdruck von mindestens 6 kPa bei 25 °C aufgelöst ist, zu einer Spinndüsenanordnung;
ausgeben der Polymerlösung in Kombination mit einem Gas zum Blasen in einer Richtung weg von mindestens einer Spinndüse in der Spinndüsenanordnung und in Gegenwart eines elektrischen Feldes, wobei die Polymerlösung durch die Spinndüse bei einer Austragsrate zwischen 6 bis 100 ml/min/Loch ausgetragen wird;
ziehen von Fasern; und
aufnehmen der Fasern auf einem Kollektor,
wobei das Lösemittel ausgewählt ist aus der Gruppe bestehend aus Pentan, Hexan, Heptan, Cyclohexan, Methylcyclohexan und Benzol.

2. Verfahren nach Anspruch 1, wobei der Dampfdruck mindestens 10 kPa bei 25 °C oder bevorzugt mindestens 20 kPa bei 25 °C beträgt.

3. Verfahren nach Anspruch 1, wobei die Polymerlösung durch die Spinndüse bei einer Austragsrate zwischen 10 bis 100 ml/min/Loch oder bevorzugt zwischen 20 bis 100 ml/min/Loch ausgetragen wird.

4. Verfahren nach Anspruch 1, wobei das Gas zum Blasen ausgewählt ist aus der Gruppe bestehend aus Luft, Stickstoff, Argon, Helium, Kohlendioxid, Kohlenwasserstoffen, Halogenkohlenstoffen, Halogenkohlenwasserstoffen und Mischungen davon.

5. Verfahren nach Anspruch 1, wobei das Gas zum Blasen eingespritzt wird mit einer Strömungsgeschwindigkeit von 50 bis 340 m/s und einer Temperatur von Umgebungstemperatur bis 300 °C.

6. Verfahren nach Anspruch 1, wobei die Fasern ein Zahlenmittel des Durchmessers von weniger als 1.000 Nanometer, bevorzugt weniger als 800 Nanometer und mehr bevorzugt weniger als 500 Nanometer aufweisen.

7. Verfahren nach Anspruch 1, wobei das elektrische Feld ein Spannungspotenzial von 10 kV bis 100 kV aufweist.

8. Verfahren nach Anspruch 1, wobei das elektrische Feld ein Coronaladungsfeld ist.

9. Verfahren nach Anspruch 1, wobei die Fasern eine Querschnittform aufweisen, die weitgehend rund ist.

10. Verfahren nach Anspruch 1, ferner umfassend Kontaktieren der Fasern mit einem sekundären Gas, das der Düsenanordnung nachgeschaltet angeordnet ist.

11. Verfahren nach Anspruch 10, wobei das Gas zum Blasen ausgewählt ist aus der Gruppe bestehend aus Luft, Stickstoff, Argon, Helium, Kohlendioxid, Kohlenwasserstoffen, Halogenkohlenstoffen, Halogenkohlenwasserstoffen und Mischungen davon.

12. Verfahren nach Anspruch 10, wobei das Gas zum Blasen eingespritzt wird mit einer Strömungsgeschwindigkeit von etwa 50 bis etwa 340 m/s und einer Temperatur von etwa Umgebungstemperatur bis etwa 300 °C.

13. Verfahren nach Anspruch 1, wobei das mindestens eine Polymer in der Polymerlösung ausgewählt ist aus der Gruppe bestehend aus Polyolefinen, Polydienen, Polystyrol, Polysulfonen, Polycarbonaten, Poly(meth)acrylaten, Celluloseestern, Polyvinylchloriden und Mischungen davon.

## Revendications

1. Procédé de filage de fibres comprenant:
la fourniture d'une solution de polymère, qui comprend au moins un polymère dissous dans au moins un solvant avec une pression de vapeur d'au moins 6 kPa à 25°C, à une filière;
la sortie de la solution de polymère en combinaison avec un gaz soufflant dans une direction s'éloignant d'au moins une buse de filage dans la filière et en présence d'un champ électrique, dans lequel la solution de polymère est déchargée par la buse de filage à un débit de décharge entre 6 et 100 ml/min/trou;
la formation de fibres; et
la récupération des fibres sur un collecteur,
dans lequel le solvant est choisi dans le groupe constitué de pentane, hexane, heptane, cyclohexane, méthylcyclohexane et benzène.

2. Procédé selon la revendication 1, dans lequel la pression de vapeur est d'au moins 10 kPa à 25°C ou de préférence d'au moins 20 kPa à 25°C.

3. Procédé selon la revendication 1, dans lequel la solution de polymère est déchargée par la buse de filage à un débit de décharge entre 10 et 100 ml/min/trou ou de préférence entre 20 et 100 ml/min/trou.

4. Procédé selon la revendication 1, dans lequel le gaz soufflant est choisi dans le groupe de: air, azote, argon, hélium, dioxyde de carbone, hydrocarbures, halocarbures, halohydrocarbures et mélanges de ceux-ci.

5. Procédé selon la revendication 1, dans lequel le gaz soufflant est injecté à une vitesse d'écoulement de 50 à 340 m/sec et une température de l'ambiante à 300°C.

6. Procédé selon la revendication 1, dans lequel les fibres ont un diamètre de fibre moyen en nombre inférieur à 1000 nanomètres, de préférence inférieur à 800 nanomètres, plus préférablement inférieur à 500 nanomètres.

7. Procédé selon la revendication 1, dans lequel le champ électrique a un potentiel de tension de 10 kV à 100 kV.

8. Procédé selon la revendication 1, dans lequel le champ électrique est un champ à chargement couronne.

9. Procédé selon la revendication 1, dans lequel les fibres ont une forme de section transversale qui est essentiellement ronde.

10. Procédé selon la revendication 1, comprenant en outre la mise en contact des fibres avec un gaz secondaire localisé en aval de la filière.

11. Procédé selon la revendication 10, dans lequel le gaz soufflant est choisi dans le groupe de: air, azote, argon, hélium, dioxyde de carbone, hydrocarbures, halocarbures, halohydrocarbures et mélanges de ceux-ci.

12. Procédé selon la revendication 10, dans lequel le gaz soufflant est injecté à une vitesse d'écoulement d'environ 50 à environ 340 m/sec et une température d'environ l'ambiante à environ 300°C.

13. Procédé selon la revendication 1, dans lequel ledit au moins un polymère dans ladite solution de polymère est choisi dans le groupe constitué de: polyoléfines, polydiènes, polystyrène, polysulfones, polycarbonates, poly(méth)acrylates, esters de cellulose, polyvinylchlorures et mélanges de ceux-ci.
